

# United States Patent

Nitz

[15] 3,641,300

[45] Feb. 8, 1972

## [54] ELECTRICAL CONTACT

[72] Inventor: Allen R. Nitz, Wauwatosa, Wis.  
[73] Assignee: Allis Chalmers Manufacturing Company, Milwaukee, Wis.  
[22] Filed: Aug. 15, 1969  
[21] Appl. No.: 850,580

[52] U.S. Cl. .... 200/166 C  
[51] Int. Cl. .... H01h 1/02  
[58] Field of Search .... 200/166 C

## [56] References Cited

### UNITED STATES PATENTS

2,417,967 3/1947 Booë ..... 200/166 C X

Primary Examiner—H. O. Jones  
Attorney—Thomas F. Kirby, Robert B. Benson and Lee H. Kaiser

## [57] ABSTRACT

In an electrical contact arrangement wherein a disconnect assembly having one or more spring loaded electrically conductive contact fingers which slidably engage and disengage from an electrically conductive stud. The fingers and stud are made of copper and the engaging surfaces are provided with a layer of silver and a layer of indium on the silver. The indium layer being on the order of 0.1–1.5 mils thick and diffused along its boundary layer to the silver by heat treatment (160° C. for 2 hours).

3 Claims, 3 Drawing Figures



PATENTED FEB 8 1972

3,641,300



Fig. 2



Fig. 1



Fig. 3

Inventor  
Allen R. Orlitz  
by Thomas F. Kirby  
Orlitz

## ELECTRICAL CONTACT

## SUMMARY OF THE INVENTION

This invention relates generally to electrical contacts. In particular it relates to silver-plated sliding contacts which have an indium coating thereon.

Some types of electrical circuit interrupters are adapted to be slid into and out of cubicles and are provided at their rear with primary disconnect assemblies which engage with studs on the bus bars to which the breaker is connectable. Each disconnect assembly typically comprises two or more spring loaded contact fingers, usually made of silver-plated copper, arranged in rows and adapted to slidably engage opposite sides of a stud, usually made of silver-plated copper. Normally, a silver plating on the order of 0.3 mils thick is sufficient to seal the copper from tarnishing when no wear is present. However, repeated withdrawal and reinsertion of the circuit breaker with respect to the cubical causes wear on the contact surfaces of the fingers of the disconnect assembly and wear on the contact surfaces of the studs. Furthermore, in chemically contaminated atmospheres where concentrations of hydrogen sulfide or sulfur dioxide are high, tarnishing of the silvered contact surfaces occurs which ultimately causes electrical failure of the disconnect assembly due to increased electrical resistance and eventual burnout.

It is known that the metal indium in its pure state or alloyed with silver or silver alloys has tarnish-resisting characteristics. U.S. Pat. No. 2,157,933 issued May 9, 1939 to Hensel and Emment and assigned to P. R. Mallory & Co. teaches electrical contacts made of silver-indium alloy. A paper entitled "A New Method for Making Low-Resistance Contacts to Aluminum" by R. W. Barnard and J. P. Pasternak presented at the Holm Seminar during Nov. 11 through 15, 1968 teaches, among other things, a connector of unspecified metal plated with indium for wedging contact with copper wire or aluminum wire and also teaches crossed aluminum and indium-plated copper wire.

However, none of these teachings offer a satisfactory solution to the problem encountered by applicant who is concerned with a disconnect contact having fingers which have a normal contact pressure of about 22.4 lbs. per square inch, which are expected to withstand at least 150 sets of insertion and withdrawal movements, which are rated at 100 amperes per finger continuous duty, and which operate at service temperature on the order of 100°C.

For example, indium plating directly on copper components is not satisfactory because contact pressure will cause the components to gradually sink through the indium layer and bear against each other thereby allowing for exposure of the copper to atmospheric conditions with consequent increases in contact resistance. Indium-silver alloys as a component material or as a coating on a component offer too high an electrical resistance for uses such as applicant's intended use and also raise cost problems. Indium in its pure state is unsatisfactory as a contact material because of its relative softness, high relative resistance and its high cost.

In accordance with the present invention the fingers of a primary disconnect assembly and a bus bar stud are made of standard electrical copper and the cooperating contact surfaces thereof are provided with a coating of silver on the order of 0.3 mils thick on which is deposited by plating or dipping a coating of indium on the order of 0.1-1.5 mils thick, after which the layer of indium adjacent the silver is partially diffused into the silver by heating for 1 to 2 hours at about 160°C.

## OBJECTS OF THE INVENTION

It is an object of the present invention to provide improved electrical contacts, particularly, primary disconnect type contacts.

Another object is to provide improved contacts which have high-current carrying capacity, relatively low-electrical resistance, and tend to resist heating.

Another object is to provide improved contacts which can withstand repeated connection and disconnection with respect to another conductive member without exhibiting undue mechanical wear and attendant resistance heating.

Another object is to provide an improved contact which comprises a silver-plated copper body on which a coating of indium is disposed and partially diffused thereinto along the boundary layer.

Another object is to provide improved disconnect contacts of the aforesaid type which comprise silvered material upon which is disposed a coating of metal selected from the group consisting of indium and gold and wherein the coating is partially diffused into the silver.

Another object is to provide an improved method for making electrical contacts which comprises the step of applying a coating of indium to a silvered material by electroplating, or chemical plating, or dipping and the step of heating said coating to effect diffusion of a portion of the indium into the silver.

Other objects and advantages of the invention will hereinafter appear.

## DESCRIPTION OF THE DRAWINGS

The accompanying drawing illustrates a preferred embodiment of the invention but it is to be understood that the embodiment illustrated is susceptible of modification with respect to details thereof without departing from the scope of the appended claims.

In the drawing:

FIG. 1 is a top view of a disconnect contact assembly associated with a bus bar stud, both in accordance with the present invention;

FIG. 2 is a side elevational view partly in section of the contact assembly and stud of FIG. 1; and

FIG. 3 is an enlarged view, partly in cross section of a contact finger of the assembly shown in FIGS. 1 and 2.

## DETAILED DESCRIPTION OF THE DRAWING

Referring to FIGS. 1 and 2 of the drawing, the numeral 10 designates a primary disconnect assembly which is mounted on an electrically conductive circuit breaker stud 12 and which is shown in engagement with an electrically conductive bus bar or cubicle stud 14. It is to be understood, for example, that stud 14 is located in a cubicle into and out of which an electrical circuit breaker can be slid and that circuit breaker stud 14 is part of such a circuit breaker. The primary disconnect assembly 10 (hereinafter called a "disconnect") serves as an electrical connection between studs 12 and 14 and is adapted to disengage from stud 14 when the circuit breaker is slid from the cubicle.

Disconnect 10 comprises a plurality of electrically conductive fingers, each of which is similar to finger 16, which are shown as arranged in two spaced-apart rows of four fingers each. The fingers in each row are biased toward each other (and against stud 14) by means of springs such as spring 18.

It is to be understood that disconnect 10 and cubicle stud 14 are rated to carry 100 amperes of current per finger during constant duty. Furthermore, they are expected to operate at service temperatures of about 100°C. Also, disconnect 10 and cubicle stud 14 are expected to withstand at least 150 sets of insertion or withdrawal movements.

Each finger 16 engages cubicle stud 14 with a normal contact pressure of about 22.4 lbs. per square inch under the action of its associated spring 18.

Referring to FIG. 3, finger 16 is fabricated of a suitable electrically conductive material 19, such as copper, and is provided with a coating 20 of silver on the order of 0.3 mils thick which, preferably, is applied by electroplating, although chemical plating or dipping could be used. In accordance with the present invention, finger 16 is further provided with a coating 22 of indium on the order of about 0.1-1.5 mil thick, which coating can be applied over the silver coating 20 by dipping or by a plating process. After coating 22 is applied,

contact finger 16 is subjected to heating to about 160° C. for from 1 to 2 hours to effect diffusion of a small amount of the indium into the silver at the interface or boundary layer between the two metals.

Referring to FIG. 3, stud 14 which slidably engages with finger 16 is also fabricated of material 24, such as copper, and is provided with a coating 26 of silver and a coating 28 of indium, except that the silver coating on stud 14 is typically only 1 mil thick.

When disconnect 10 is moved into engagement with cubicle stud 14, each contact finger 16 makes sliding engagement with the cubicle stud, as FIG. 3 shows. The indium coating 22 on finger 16 and the indium coating 28 on stud 14 are soft enough to be somewhat displaced because of the spring pressure. Therefore, the undiffused indium serves as an electrically conductive tarnish resistant lubricant between contact finger 16 and stud 14. The diffused indium inhibits scratching, marring or scoring on the silver plating on the copper subsurfaces and improves the tarnish resistance of the silver plating. Thus, the indium effectively protects the silver plating against mechanical damage. Even though the indium has a higher coefficient of electrical resistance than either silver or copper it does not interfere with the electrical conductivity of the connection between the finger 16 and the stud 14 for two reasons. First, the contact pressure is such as to cause the indium coating to be squeezed to a dimension thinner than the normal plating thickness of the indium. Second, because of the relative softness of the indium it tends to flow in such a manner as to make contact with a greater area of the surface of finger 16. In this way point contact, line contact, or small surface area contact is avoided and the higher coefficient of resistance of the indium is compensated for by the greater contact area.

When finger 16 and stud 14 are separated, the lubricating effect of the indium prevents or inhibits contact wear and the indium tends to assume its normal uniform coating charac-

teristics.

In the embodiment of the invention shown, the fingers 16 and the cubicle stud 14 are shown as having coatings of silver and indium. It is to be understood, however, that the finger alone may be provided with the silver and indium coating and good electrical contact results. Furthermore, although a disconnect assembly is shown, it is apparent that other types of contacts could be made in accordance with the present invention.

10 The embodiments of the invention in which an exclusive property or privilege is claimed are defined as follows:

1. In a slidable electrical contact, an electrically conductive body having a contact region subject to tarnishing,

15 a layer of silver on said contact region of sufficient thickness to seal said contact region against tarnishing, and a layer of indium of a thickness between about 0.1 and about 1.5 mils thick on said layer of silver, said layers of silver and indium being diffused along their boundary layer.

20 2. A contact according to claim 7 wherein the contact region has a radius of curvature and is adapted to slidably engage another conductive body.

25 3. In combination, a pair of slidably engageable electrical contacts having tarnishable contact regions thereon, at least one of said contacts having a contact region which has a radius of curvature, a layer of silver on each of said contact regions of sufficient thickness to seal said surfaces against tarnishing, and a layer of indium of a thickness between about 0.1 and about 1.5 mils thick on each of said layers of silver, said layers of silver and indium being diffused along their boundary layers.

\* \* \* \* \*

40

45

50

55

60

65

70

75